

Aug. 4, 1931.

R. E. LOWE

1,817,888

PROTECTIVE COATING (ALBORIZING)

Filed Sept. 15, 1927

*Fig. 1.*



*Fig. 2.*



Inventor  
RUSSELL E. LOWE

By his Attorney

Edmund G. Borden

## UNITED STATES PATENT OFFICE

RUSSELL EDMUND LOWE, OF NEW YORK, N. Y., ASSIGNOR TO DOHERTY RESEARCH COMPANY, OF NEW YORK, N. Y., A CORPORATION OF DELAWARE

## PROTECTIVE COATING (ALBORIZING)

Application filed September 15, 1927. Serial No. 219,660.

It has long been an objective of those engaged in engineering to make iron and steel articles capable of withstanding comparatively high temperatures without scaling 5 while retaining the full strength and heat conductivity of the ferrous metal. Articles such as pipe stills, recuperators and the like are required to transmit heat while subjected to high temperatures under oxidizing 10 conditions, often under high pressures. If the tubes of such devices are oxidized to form a scale the fraction of an inch thick, the strength of the tubes is materially weakened and they must be replaced at a considerable expense. It has been proposed to coat iron and steel with coatings of various materials with a view to preventing scaling of the iron or steel. Among other materials, aluminum has been proposed as a 15 protective coating for this purpose. The so-called calorized articles are composed of ferrous bodies having a ferro-aluminum coating formed by heating the iron or steel articles in powdered aluminum under a hydrogen atmosphere and at a considerable 20 temperature. However, in order that the calorizing process be effective in preventing scaling, so much aluminum is alloyed with the iron or steel body of the article as to 25 weaken it materially when exposed to high temperature. Moreover, the calorizing process has not been worked out as to its application to articles of large size or of unwieldy character. 30

It has been proposed also to use thin coatings of aluminum metal on iron articles for decorative purposes and for protection against rust at ordinary temperatures. The thin aluminum coatings used for the purposes just mentioned, however, have not been of a character to resist more than a moderate heat or to protect the iron or steel beneath from oxidation. 35

It is one object of the present invention 40 to provide a ferrous article having an aluminum coating and capable of both withstanding an oxidizing atmosphere at high temperatures without scaling and withstanding high pressures. 45

Another object of the invention is to pro-

vide a method of making the aluminum coated article.

Further objects and advantages of the present invention will be apparent to those skilled in the mechanical and chemical arts 55 from the following description taken with the accompanying drawings in which

Fig. 1 illustrates an article embodying the present invention;

Fig. 2 is a detail view illustrating a portion of the article of Fig. 1 as it appears under a magnification of two hundred diameters.

In the drawings, 10 is a tube of iron or steel of the kind used in boilers, pipe stills, recuperators and/or like structures. The outer surface of tube 10 is covered by a relatively thin but tough imperforate glazed layer or coating 12 inert to oxygen at 1400° F. and below. The coating 12 is alloyed with the metal at the surface of the tube 10 so that it adheres firmly thereto. Alloying between the tube 10 and the coating 12 is indicated in the drawing by the irregular line or surface of jointure 14. Line 14 lies within the original surface of tube 10. While the coating 12 is preferably quite thin, blistering occurring if it is thickened beyond a certain point, it should, preferably be of sufficient thickness to prevent the formation of apertures or pinholes under high temperature conditions. Said apertures cause the ferrous body of an article to be attacked by oxygen. The coating 12 is preferably about .002 inch thick, the thickness being taken as an average over the entire coating. Also, the coating 12 should be alloyed to the body of article 10 in order to prevent scaling or flaking of coating 12. 55

The thickness of the protective coating 12, may, however, range from .001 inch to .02 inch within the present invention, although no practical advantage has been found in employing coatings over .002 inch thick. Coatings averaging much less than .002 in thickness will be apt to prove imperfect through the presence of pinholes, while heavier coatings may blister in the process of formation. An additional dis-

advantage inherent to excessively heavy coatings, even if the same have been successfully applied, lies in their tendency towards disruption through diminution of their elasticity and the fact that there exists a difference in co-efficient of expansion between the coating and unaffected steel. The thickness of coating 12 should be superficial with respect to the wall of the ferrous portion of article 10 in order that the ferrous wall or body retain its original strength. The coating 12 has a dull blue-gray color due to a slag glaze 16 on its outer surface and is composed of slag and alloy, the slag occurring principally as separate particles in the alloy. In the drawings, the slag particles in coating 12 are indicated by dots 18 in Fig. 2, the alloy being indicated at 20. The outer portion of the coating 12 is high in slag and low in metal or alloy and the percentage composition of coating 12 varies in passing inwardly therethrough to an inner surface which is low in slag and high in metal. The slag in coating 12 is composed of alumina and iron oxide combined with borax. The alloy in coating 12 is an iron-aluminum alloy and is richest in iron at the line or surface of juncture 14.

The article according to the present invention and above described is formed preferably by the following process which also forms part of the present invention:

The ferrous surface to be protected is thoroughly cleaned, usually by pickling, and drying. A protective coating is then formed on the dry surface. For this purpose preferably a liquid carrier is prepared containing aluminum powder or flake in suspension. The carrier liquid, if used, must have sufficient fluidity to spread easily, but it must have sufficient body to carry the metallic aluminum flake and a flux in suspension without agglomeration so that an even thickness of aluminum coating may be formed. The mixture must not, however, be so fluid that it spreads too thin and thereby deposits too little aluminum per unit area of surface to be protected, or so thick that too much aluminum is deposited per unit area of ferrous surface. The carrier must also volatilize under heat without excessive formation of undesirable material, such as carbon, and without peeling or blistering. It has been found that a suitable liquid carrier for use in the present process is one formed by mixing four parts of rectified spirits of turpentine with one part acid-free spar varnish. Turpentine and spar varnish are both well known articles of commerce. The spar-varnish of commerce while of varying composition according to the maker, yields an elastic non-perforate dense coating or glaze when dry and imparts these desirable characteristics to the deposit formed by the liquid when dried

on a surface to be coated according to the present invention. Benzene (benzol), and spar varnish, cellulose and a cellulose solvent, and a solution of rubber in a rubber solvent are examples of other liquids that may be used in the present process as carriers for aluminum flake in place of the said turpentine-varnish mixture. Amyl acetate is an example of a suitable cellulose solvent and acetone, acetone and ether, and benzene are examples of rubber solvents which may be used in making cellulose or rubber solutions for use as carrier liquids when practicing the present invention. The ingredients of the carrier must be substantially free from water.

The aluminum for forming the protective coating is incorporated into the liquid carrier, preferably in the form of aluminum flake. It has been found that the characteristics of the coating formed depend in large measure upon the size of the aluminum flake which is used. If the very fine sizes of aluminum powder or flake are used, the coating produced is unsatisfactory; either being too thin or containing so much alumina (oxide of aluminum) as to form holes in the coating. It therefore fails under high temperature. On the other hand, if the flake is too coarse, it settles out of the carrier liquid and does not make a uniform coating. #46 commercial aluminum flake is satisfactory. The aluminum flake is incorporated into the liquid carrier and with it is incorporated a flux material. The material used as flux must have certain characteristics. It must be substantially dry under the conditions of the process. If water is driven off during the operation of coating, the coating is blistered and its aluminum content more or less completely oxidized and no protection to the underlying metal is afforded. Also the flux material must melt at a low enough temperature to protect the aluminum flake from oxidation while the flake is alloying with the ferrous body. The flux material must have a good solvent action on iron oxide and a solvent action, although a less one, on the aluminum oxide. The only known satisfactory flux for use in the present process is finely divided anhydrous fused borax. Ordinary hydrous borax is not suitable for the reason that it causes blisters in the coating.

When the aluminum flake and the flux have been incorporated into the liquid carrier, (assuming a carrier is used), the mixture is applied evenly to the cleaned surface of the ferrous article to have the protective coating formed thereon. The mixture is allowed to dry and resulting layer of dried liquid carrier, aluminum flake and flux is then heated quickly to the melting point of the flux and the heating continued until the desired adherent protective coating is

formed. A high temperature flame may be used for heating the dried mixture as just described. During the heating to form the protective coating, the dense nonperforate elastic glaze formed by the dried liquid carrier serves to partly protect the finely divided aluminum from oxidation until the flux melts, the melted flux then partly protecting the aluminum flake from oxidation.

10 The organic carrier liquid is completely driven off or burned by the heating of the dried mixture in the formation of the desired protective coating.

By way of example, a specific manner of 15 practising the process for producing the protective coating on ferrous materials according to the present invention is as follows:

A convenient quantity of aluminum for forming the basis of a batch of coating material is first taken. Fourteen grams of No. 46 chemically pure aluminum flake is a suitable amount and character of material for this purpose. A typical screen analysis of No. 46 aluminum flake shows approximately 25 that two-tenths of one percent of #46 flake is retained on a screen having 100 meshes to the inch; of the material passing through 100 mesh screen 1.6% is retained on a 120 mesh screen; of the material passing 120 mesh screen 21.2% is retained on a screen having 140 mesh per square inch; of the material passing the 140 mesh screen, 6.5% is retained on a 160 mesh screen; of the material passing the 160 mesh screen, 1.8% 35 is retained on the 180 mesh screen; of the material passing the 180 mesh screen 23.5% is retained on the 200 mesh screen; and 45.2% passes the 200 mesh screen. It will be noted that greater than 50% of the material is coarser than 200 mesh. The invention is not limited to No. 46 flake, or to flake of the same fineness. It has been found that #20 flake is too coarse and #99 flake or powder is too fine for best results. Sizes 45 between Nos. 20 and 99 flake may be usefully employed. The reasons why the flake or powder used must lie within certain limits of fineness appear above. With the 14 grams of flake are incorporated preferably 50 14 grams of fused anhydrous borax, 200 mesh or finer, and the whole then mixed with 80 cubic centimeters of rectified spirits of turpentine and 20 cubic centimeters of acid-free spar varnish. After the ferrous 55 surface has been prepared as mentioned above, the mixture containing the ingredients substantially as just stated, or their equivalents, is then flowed over the surface or otherwise applied thereto in such manner as to uniformly and thoroughly coat the entire surface. The mixture, when of the proper consistency has a distinctly "tacky" nature, said consistency materially aiding in suspending the borax and the 65 metal flake and in causing adherence of the

mixture to the metallic surface to be coated. A batch of the mixture containing 14 grams of 70 46# aluminum flake, 14 grams of finely divided fused borax, 80 cc of rectified spirits of turpentine and 20 cc acid-free spar varnish coats when used in the present process about 3 sq. ft. of surface. The dried deposit and also the finished protective coating therefore contain about 4.0 grams of aluminum per sq. ft. After the mixture has been 75 applied to the article, it is then set aside to dry, preferably at atmospheric temperature, until the mixture is distinctly hard. The hardening of the liquid mixture has been found to take about an hour under ordinary 80 conditions. After the mixture has hardened the external layer formed on the article is about .002 inches in thickness. The article is then heated to drive off the liquid vehicle from the mixture, to fuse the flux and aluminum, and to form the coating 12. Preferably the heating of the article for the 85 purposes just mentioned is performed by "flashing" with an oxy-acetylene torch using a broad flame about 1 inch in diameter until the section under heat treatment assumes a dull blue gray color. Actual temperature attained during flashing=1400-1550° F. In the language of the operatives, the coating is then properly "cooked". The 90 desired color is acquired in a very short time and therefore the torch may be kept moving slowly and the "flashing" made continuous. It is necessary to the formation of a satisfactory coating 12 that the temperature of the flux be brought to its melting point very quickly so that it will fuse on the aluminum grains and protect them from over oxidation. It has been found, for instance, that the flame of an ordinary Bunsen burner does not melt the flux quickly enough for good 95 results when used in the open air. The result of heating too slowly is to cause so much of the aluminum flake or powder to oxidize before it melts and alloys with the ferrous surface that the resulting coating contains holes and is of a friable and blistery character unless the steel being treated is of very thin section. After the flux has fused, it not only protects the aluminum, but 100 dissolves the iron and aluminum oxides on the surfaces in contact and so promotes the alloying of the aluminum to the ferrous body. Of course, the coating 12 does not adhere properly to the body 10 unless the aluminum alloys with the body 10, at least 105 at the surface of the body. The aluminum alloys with the iron to the desired degree under the conditions mentioned above.

The articles according to the present invention retain their full strength under very severe heat conditions. This is borne out by a comparative experiment using calorized tubes and tubes according to the present invention. The calorized tubes and 110

115

120

125

130

those treated by the present process were of the same original dimensions and material. The calorized tubes were exposed to an internal air pressure of 500 lbs. while maintained in an oxidizing atmosphere at a temperature of 1200° F. The calorized tubes under the conditions mentioned softened and swelled after three days. The tubes according to the present invention, however, were subjected to an internal air pressure of 1000 lbs. while surrounded by an oxidizing atmosphere for six months at temperatures ranging between 1000° F. and 1500° F., but without showing signs of distress. The coating, however, began to blacken when held for a time at temperatures above 1400° F. While an article according to the present invention may be held at 1400° F. for some time without showing signs of oxidation, the ordinary upper working limit of temperature for articles according to the present invention over periods of time as long as six months is 1200° F.

It will be understood that the tubes according to the present invention which were tested as above described by the present process both internally and externally. It is one of the advantages of the present process that a protective coating may be formed on both the inner and outer surfaces of hollow articles of moderate thickness and at the same time. In order to form a protective coating on both inner and outer surfaces to an article it is necessary only to flow the liquid mixture of the character described in the above example over both surfaces to form a deposit containing the aluminum and flux. When the deposit is dried as above described it may then be flashed by the high temperature flame, the flame being applied to either surface as is most convenient, the resulting heating producing a protective coating according to the present invention on both surfaces simultaneously.

While it is preferred to use a liquid vehicle or carrier to apply the aluminum powder or flake and borax flux to the surface on which a protective coating according to the present invention is to be formed, the use of a liquid vehicle or carrier may be omitted. A suitable method of forming a protective coating according to the present invention when no liquid carrier is employed is as follows: The ferrous surface to be coated is cleaned and then an even layer of aluminum powder or flake of suitable size is sifted or otherwise spread on said surface. Said layer should contain a suitable weight of aluminum per square ft. of surface. As above indicated, .15 oz. of aluminum per sq. ft. of surface to be coated is a suitable weight of aluminum, but the invention is not limited to this. Powdered anhydrous

borax may then be sifted or spread evenly in other ways over the layer of aluminum powder or flake. The borax powder is used in sufficient quantity to cover the aluminum and to protect it in large measure against oxidation during the subsequent heating period. A weight of borax powder equal per sq. ft. to that of the aluminum is a suitable amount of borax, but the invention is not limited to this. After the aluminum and borax powders have been applied to the surface to be coated, the ferrous article is then heated quickly to melt the borax and to form a protective aluminum containing coating which alloys with the surface of the ferrous article. The heating of the article to be coated when the liquid carrier is omitted may be performed in an enameling furnace. Of course, a blast flame cannot be applied directly to the surface carrying the powdered aluminum and borax since the blast would scatter the powders. In case of a thin sheet however, a blast flame, such as that from an oxy-acetylene flame, can be applied to the underside of a sheet whose top horizontal surface carries a layer of powdered aluminum and powdered anhydrous borax to melt the borax and aluminum and to form the desired protective coating on the upper surface of the sheet. Moreover, I find that, when desired, coatings of a thickness up to .02 inches can be built up by spraying, provided the metal has been preheated to and is maintained at such temperature that the liquid vehicle in which the aluminum flake is suspended is rapidly volatilized. It will be evident also from the foregoing that I am not limited to the use of the liquid carriers mentioned above, other liquids having been used as carriers in forming aluminum coatings for decorative and like purposes.

As above indicated, it is preferred to use aluminum powder or flake when operating according to the present invention at the rate of approximately .15 oz. of aluminum per sq. ft. of surface to be coated. A coating according to the present invention and having .15 ounces aluminum per sq. ft. protects against scaling as above mentioned. However, useful results as to protection from scaling are obtained when using as little as .05 ounces of aluminum per sq. ft. and as much as .25 ounces per sq. ft. of surface to be coated. Moreover, the amount of borax used need not be equal to the amount per sq. ft. of surface to be coated, it being practicable within the present invention to protect against scaling when varying the ratio between the borax and the aluminum from as much as two parts of borax to one of aluminum to as little as one of borax to two of aluminum; provided, however, the amount of borax does not fall

below .05 ounces per sq. ft. when making an anti-scaling coating.

In the foregoing description, the present invention is disclosed as applied to iron or 5 ferrous articles. It will be understood however that the invention is not limited to protecting the surfaces of articles composed essentially of iron, but may be applied likewise to alloys containing considerable 10 amounts or percentages of iron, such for instance, as nickel-steel, chrome-steel, manganese-steel, vanadium-steel, and molybdenum-steel.

Also it will be evident from the foregoing 15 that one aspect of the present invention involves the discovery of the advantages flowing from the use of anhydrous fused borax as a flux when forming aluminum containing coatings on surfaces of ferrous articles 20 and that while of particular usefulness in protecting iron against high temperatures, the coatings formed when using a flux of fused anhydrous borax may be used also for decorative and rust preventive purposes. 25 When aluminum containing coatings are to be formed for decorative and/or rust preventive purposes only, the quantity limits stated above do not apply.

Having thus described my invention, I 30 claim:

1. The process of forming a protective coating on a ferrous surface including covering the ferrous surface to be protected with a mixture of aluminum flake of a size 35 between those of Nos. 20 and 99 and finely divided anhydrous fused borax in a liquid vehicle, said vehicle holding the flake and borax in suspension without agglomeration while forming a tacky mixture, drying said 40 mixture, and heating said dried mixture rapidly enough to coat the aluminum particles with fused borax before a material percentage of the aluminum flake has been converted into oxide to drive off the dried 45 vehicle and alloy the aluminum with the ferrous body in a thin layer forming an imperforate coating having a glazed surface.

2. The method of forming a protective coating on a ferrous article comprising covering the surface of said article to be coated with a uniform deposit containing between .05 oz. and 1.25 oz. of divided aluminum per 50 square foot of said surface, said deposit containing also anhydrous borax, and alloying said aluminum with said surface by heating under conditions deterrent to the oxidation of said aluminum.

3. The method of forming a protective coating on a ferrous article comprising 55 cleaning the surface to be coated, covering said surface with a uniform layer containing approximately .15 oz. of finely divided aluminum per square foot and an approximately equal amount of finely divided anhydrous borax, and alloying said aluminum

with said surface under conditions deterrent to the oxidation of said aluminum.

4. The method of forming a protective coating on a ferrous article comprising 60 cleaning the surface to be coated, flowing onto said surface a mixture of a carrier liquid holding in suspension finely divided aluminum and finely divided anhydrous borax and drying said liquid on said surface to form a deposit containing uniform 65 amounts of aluminum and borax per square foot of surface, and heating said deposit under conditions deterrent to oxidation of said aluminum to alloy said aluminum to 70 said surface and to form a uniform coating 75 thereon.

5. The process of forming a protective coating on a ferrous surface including covering said surface with a mixture of aluminum flake of a size between those of Nos. 80 85 20 and 99 and finely divided anhydrous fused borax in a liquid vehicle, said vehicle holding said flake and said borax in suspension without agglomeration while forming a tacky mixture and containing turpentine and spar varnish, drying said mixture on said surface to form a uniform deposit, and heating said deposit rapidly enough to coat the aluminum particles with fused 90 borax before a material percentage of the 95 aluminum flake has been converted into oxide, to drive off the dried vehicle and to alloy the aluminum to said surface in a thin imperforate layer.

6. In a method of forming an aluminum 100 containing coating on the surface of a ferrous article, the step including heating a layer of aluminum on said surface in the presence of finely divided anhydrous fused borax.

7. In the manufacture of a coated ferrous article, the improvement comprising the steps of covering the ferrous surface to be coated with a uniform layer of aluminum flake and finely divided fused borax, said 110 layer containing between .05 ounces and .15 ounces of aluminum per square foot and between .05 ounces and .15 ounces of borax per square foot, and quickly heating said layer to 1400° F. under conditions deterrent to 115 oxydation to alloy said aluminum to said surface and to form an aluminum containing coating inert to oxygen at 1200° F. over long periods.

In testimony whereof I affix my signature.

RUSSELL EDMUND LOWE.